

N. C. COTABISH.  
WATER METER.  
APPLICATION FILED OCT. 11, 1915.

1,182,354.

Patented May 9, 1916.

FIG. 1



FIG. 3



FIG. 2



WITNESS  
*H. G. Grover*

INVENTOR.  
NELSON C. COTABISH  
BY *Ira J. Adams*  
ATTORNEY

# UNITED STATES PATENT OFFICE.

NELSON C. COTABISH, OF LAKewood, OHIO.

## WATER-METER.

1,182,354.

Specification of Letters Patent.

Patented May 9, 1916.

Application filed October 11, 1915. Serial No. 55,184.

*To all whom it may concern:*

Be it known that I, NELSON C. COTABISH, a citizen of the United States, residing at Lakewood, in the county of Cuyahoga and 5 State of Ohio, have invented a certain new and useful Improvement in Water-Meters, of which the following is a full, clear, and exact description.

My invention relates to water meters and 10 the object is to construct the piston-disk of such meters of a material that is insensitive to temperature changes and will retain its shape regardless of the temperature of the water passing around it.

15 Referring to the drawings:—Figure 1 represents more or less conventionally a typical water meter with certain parts broken away to show the special feature of my invention. Fig. 2 represents a top view 20 of the meter shown in Fig. 1. Fig. 3 represents a piston-disk shown in the cut-away portion of Fig. 1.

Referring to Fig. 1, a metallic casing 1 is provided with inlet and outlet tubes 2 25 and 3 for the passage of water therethrough. A piston disk 5, having two hemispherical bearing members 6, oscillates in a well known way within the water chamber 7 due to the passage of the water therethrough. A pin 30 8 is secured to the central part of the upper bearing member 6 and the disk 5 in such a way that it rotates a toothed wheel 9 as the disk oscillates under the propelling action of the water. The rotation of the wheel 9 35 actuates the registering hands 10 (Fig. 2) by means of a train of appropriate gearing and thereby registers the volume of water that has passed through the meter.

The general arrangement of the meter is 40 the same as that commonly used and needs no further explanation.

It has been the universal practice, as far as I am aware, to construct the piston-disk 5 of hard rubber or other rubber compound 45 on account of its non-corrodible character. Hard rubber, however, cannot stand the effects of heat and will warp and become otherwise distorted whenever subjected to a material increase of temperature above the 50 normal limit. Inasmuch as water meters are often subjected to the action of hot water through carelessness of the consumer in controlling hot water appliances, there has been frequent trouble from warped pis- 55 ton-disks in the meter. It has been pro-

posed to decrease this difficulty by mixing graphite with the rubber compound before vulcanization, with the idea that this would lessen the tendency of the rubber disk to warp when heated. Such proposal, however, has not resulted in material improvement, as the rubber-graphite composition will warp if subjected to water or steam slightly above 212°. Inasmuch as temperatures in excess of this are frequently attained, the graphite rubber disk has not been satisfactory. Again, rubber-graphite disks are weak and quite brittle so that they often break in the regular operation of the meter or during handling prior to installing in the 70 meter.

On experimentation, I have found that the piston-disk can be made of carbon flour held together by pitch, tar or other carbonaceous binder, which on coking in an appropriate furnace, rigidly binds the carbon particles together. The carbon disk should contain no rubber, as the latter will cause it to warp as in prior disks. When made entirely of carbon the disk is very strong and 80 is absolutely unaffected by temperature changes in the water passing through the meter. Carbon disks are therefore peculiarly suited for the purpose to which I apply them, as they are non-corrodible and 85 entirely unaffected by either hot or cold water.

To make the disk I mix fine carbon flour, such as that obtained from coke or lamp-black for example, with sufficient pitch or 90 tar to render it plastic under heat when molded. Ordinarily I mix about 85 to 90 per cent. of carbon flour with 15 to 10 per cent. of powdered pitch, although other proportions may be used, and after thoroughly 95 mixing the two, the conglomerate is placed in a properly shaped mold and submitted to hydraulic pressure to densely compact the same. During this operation the mold is heated by appropriate means to a high 100 enough temperature to soften the hard pitch and cause it to flow and envelop carbon particles. The disk is then removed from the mold and baked in a furnace to a temperature that will set the binder and cause the 105 carbon particles to be rigidly coked together. This temperature will vary depending upon circumstances, but ordinarily will be in the neighborhood of 900° C.

Instead of using pitch as the binder, I 110

may use tar or saccharin solutions, which will carbonize and coke the carbon particles together in the same way as has been described in reference to the powdered pitch.

5 Having described my invention, what I claim is:—

1. In disk water meters having registering mechanism, a meter casing and a piston-disk in said casing adapted to operate said registering mechanism said disk consisting

of carbon particles held together by a coked binder.

2. As an article of manufacture a piston-disk for disk water meters consisting of carbon particles held together by a coked 15 binder.

In testimony whereof, I hereunto affix my signature.

**NELSON C. COTABISH.**